

# UNITED STATES PATENT OFFICE.

WALTER O. SNELLING, OF ALLENTOWN, PENNSYLVANIA, ASSIGNOR TO TROJAN POWDER COMPANY, OF NEW YORK, N. Y., A CORPORATION OF NEW YORK.

## EXPLOSIVE.

1,386,440.

Specification of Letters Patent.

Patented Aug. 2, 1921.

No Drawing. Application filed February 11, 1920, Serial No. 357,900. Renewed January 21, 1921. Serial No. 439,055.

*To all whom it may concern:*

Be it known that I, WALTER O. SNELLING, a citizen of the United States, and resident of Allentown, Lehigh county, Pennsylvania, 5 have invented certain Improvements in Explosives, of which the following is a specification.

My invention relates to explosives, and particularly to solid organic nitrate explosives capable of use for military purposes, and its object is the production of an improved explosive which shall be highly insensitive to shocks and yet be capable of detonation by means of a suitably powerful 15 initial priming or booster charge, and shall possess other characteristics advantageous in a military explosive.

My improved explosive in its preferred form comprises nitrostarch, an inorganic 20 nitrate, a desensitizing agent, and such additional ingredients as are ordinarily employed in making up explosive mixtures of this general type. While I prefer to employ nitro starch as the organic nitrate, other 25 solid organic nitrates may be employed, such as nitro cellulose, nitrated ivory nut, or nitrated sugar.

My preferred inorganic nitrate is ammonium nitrate, but other nitrates may be 30 successfully employed, such for example as the nitrates of sodium, potassium or barium, or mixtures of such nitrates, and other inorganic chemical compounds of high available oxygen content may be employed such 35 as alkali metal chlorates, perchlorates and the like.

As a desensitizing agent I use oil, preferably a heavy lubricating oil, although 40 lighter mineral oil may be used, as well as animal and vegetable oily materials such, for example, as lard oil and cotton-seed oil, or mixtures of oils, natural or artificial. Such a natural mixture of oils as is represented by gas-tar may be used, if strongly 45 acid components are first removed or neutralized.

While small proportions of oil have heretofore been used in nitro-starch mixtures for such purposes as waterproofing or to give 50 consistency, it has not, so far as I am aware, been proposed to use oil, or oily material, in large proportions relative to the nitro-starch to serve as a sole desensitizing agent. I have discovered that by the use of oil in

amounts ranging above 10% of the weight 55 of the nitro-starch in the nitro-starch-organic-nitrate mixture, an explosive can be obtained which while being remarkably insensitive can yet be detonated by means of a suitable booster charge, with violent explosion.

My invention may be utilized in a large range of mixtures varying in nitro-starch content—the following table indicating the 65 proportions of oil used:

In mixtures which contain 20% of nitro-starch, I may use not less than 2% of oil and not more than 5% of oil, my inorganic nitrates, anti-acid ingredients and other 70 added materials varying within the range of 75% to 78%.

In mixtures which contain 30% of nitro-starch, I may use not less than 3% of oil, and not more than 7½% of oil, my inorganic 75 nitrates, anti-acid ingredients and other added materials varying within the range of 62½% to 67%.

In mixtures which contain 40% of nitro-starch, I may use not less than 4% of oil, and not more than 10% of oil, my inorganic 80 nitrates, anti-acid ingredients and other added materials varying within the range of 50% to 56%.

In the mixtures which contain 50% of nitro-starch, I may use not less than 5% of 85 oil, and not more than 12½% of oil, my inorganic nitrates, anti-acid ingredients and other added materials varying within the range of 37½% to 45%.

In mixtures which contain 60% of nitro-starch, I may use not less than 6% of oil, and not more than 15% of oil, my inorganic nitrates, anti-acid ingredients and other 90 added materials varying within the range of 25% to 34%.

In mixtures which contain 70% of nitro-starch, I may use not less than 7% of oil, and not more than 17½% of oil, my inorganic 95 nitrates, anti-acid ingredients and other added materials varying within the range of 12½% to 23%.

In general, the amount of oil which I use is not less than 10% nor more than 25% of the amount of nitrostarch which I use, the difference between the combined weights 100 of the nitro-starch and the oil being an inorganic nitrate or a mixture of inorganic nitrates, altogether with minor amounts of

anti-acid and stabilizing ingredients. Where another solid organic nitrated body is substituted for nitro-starch the range of percentages of oil and nitrated body are the same as in the nitro-starch.

By employing the ingredients in the proportions indicated, explosives of great value for military purposes may be obtained. Because of the extreme insensitiveness to 10 shocks,—they are insensitive to even a No. 8 detonating cap—they can be safely used for aerial drop bombs, as well as for sea mines, torpedoes, high explosive shell and similar military uses. While inert to even such 15 shocks and blows as would be represented by the impact of a shell with armor plate or a cement wall, they may still be detonated, with very violent explosion, by means of a suitable booster charge.

20 I claim:—

1. An explosive containing nitro-starch desensitized by the presence of oil in an amount of not less than 10% of the nitro-starch.
- 25 2. An explosive comprising nitro-starch and an inorganic oxidizing agent, and a desensitizing agent consisting of oil in an amount of not less than 10% of nitro-starch.
3. An explosive comprising nitro-starch,

an inorganic nitrate, and a desensitizing agent consisting of oil in an amount of not less than 10% of nitro-starch.

4. An explosive comprising nitro-starch, an inorganic nitrate, and oil in an amount of not less than 10% nor more than 25% of the 35 nitro-starch.

5. An explosive comprising nitro-starch, an inorganic nitrate, and a heavy lubricating oil in an amount of not less than 10% of the nitro-starch.

40 6. An explosive comprising nitro-starch from 20% to 70%, an inorganic nitrate, and oil from 2% to 17½%, said oil constituting not less than 10% nor more than 25% of the nitro-starch.

45 7. An explosive containing 50% of nitro-starch; 7½% of heavy mineral oil; and 42½% of an inorganic oxidizing agent.

8. An explosive containing 50% of nitro-starch; 7½% of heavy mineral oil; and 42½% 50 of an alkali metal perchlorate.

9. An explosive comprising nitro-starch, an inorganic nitrate, and a desensitizing oil in sufficient amount to prevent detonation with a No. 8 detonating cap while permitting the detonation by means of a suitable booster charge.

WALTER O. SNELLING,